



US006830604B2

(12) **United States Patent**  
Grearson et al.

(10) Patent No.: **US 6,830,604 B2**  
(45) Date of Patent: **Dec. 14, 2004**

(54) **TOOL FOR DRILLING/ROUTING OF  
PRINTED CIRCUIT BOARD MATERIALS**

(75) Inventors: **Alistair Grearson**, West Midlands (GB); **John Aucote**, Warks (GB)

(73) Assignee: **Sandvik AB**, Sandviken (SE)

(\*) Notice: Subject to any disclaimer, the term of this patent is extended or adjusted under 35 U.S.C. 154(b) by 206 days.

(21) Appl. No.: **10/278,073**

(22) Filed: **Oct. 23, 2002**

(65) **Prior Publication Data**

US 2003/0047031 A1 Mar. 13, 2003

**Related U.S. Application Data**

(62) Division of application No. 09/486,586, filed as application No. PCT/SE98/01574 on Sep. 4, 1998, now Pat. No. 6,521,172.

(30) **Foreign Application Priority Data**

Sep. 5, 1997 (SE) ..... 9703204

(51) **Int. Cl.** <sup>7</sup> ..... **C22C 1/10**

(52) **U.S. Cl.** ..... **75/236**

(58) **Field of Search** ..... 75/232, 236

(56) **References Cited**

**U.S. PATENT DOCUMENTS**

|             |         |                     |
|-------------|---------|---------------------|
| 3,994,716 A | 11/1976 | Huppmann et al.     |
| 4,093,450 A | 6/1978  | Doyle et al.        |
| 4,469,505 A | 9/1984  | Cheresnowsky et al. |
| 4,539,041 A | 9/1985  | Figlarz et al.      |
| 4,574,011 A | 3/1986  | Bonjour et al.      |
| 5,476,531 A | 12/1995 | Timm et al.         |
| 5,482,530 A | 1/1996  | Höhne               |

|              |          |                             |
|--------------|----------|-----------------------------|
| 5,603,075 A  | 2/1997   | Stoll et al.                |
| 5,658,678 A  | 8/1997   | Stoll et al.                |
| 5,802,955 A  | 9/1998   | Stoll et al.                |
| 6,015,447 A  | 1/2000   | Görge et al.                |
| 6,086,980 A  | * 7/2000 | Foster et al. .... 428/212  |
| 6,413,293 B1 | * 7/2002 | Grearson et al. .... 75/240 |
| 6,521,172 B2 | * 2/2003 | Grearson et al. .... 419/18 |

**FOREIGN PATENT DOCUMENTS**

|    |           |         |
|----|-----------|---------|
| AT | 268706    | 2/1969  |
| DE | 2 225 896 | 12/1972 |
| DE | 27 19 532 | 11/1977 |
| GB | 622041    | 4/1949  |
| GB | 1309634   | 3/1973  |
| WO | 92/13112  | 8/1992  |
| WO | 92/18656  | 10/1992 |

**OTHER PUBLICATIONS**

V. A. Tracey et al., "Development of Tungsten Carbide–Cobalt–Ruthenium Cutting Tools for Machining Steels", vol. 82, No. 1, 1998, XP000574252, pp. 281–292.

B. Zetterlund, "Cemented Carbide in High Pressure Equipment", *High Pressure Engineering*, vol. 2, 1997, pp. 35–40.

\* cited by examiner

*Primary Examiner*—Daniel Jenkins

(74) *Attorney, Agent, or Firm*—Burns, Doane, Swecker & Mathis, L.L.P.

(57) **ABSTRACT**

A dense cemented carbide product is described. The product is manufactured from WC with a grain size between 0.1 and 0.4  $\mu\text{m}$ , fine grain size cobalt and ruthenium powders. The product is used in PCB machining operations where the addition of 10–25% Ru to the binder phase offers up to 25% wear resistant increases and up to 100% increase in chipping resistance in PCB routing compared to conventional materials (6% cobalt and 0.4  $\mu\text{m}$  grain size).

**5 Claims, No Drawings**

## 1

TOOL FOR DRILLING/ROUTING OF  
PRINTED CIRCUIT BOARD MATERIALS

This Application is a Divisional Application of Ser. No. 09/486,586 filed 15 May 2000, now U.S. Pat. No. 6,521,172 which is a 371 of PCT/SE98/01574 filed 4 Sep. 1998.

The present invention relates to a tool for drilling/routing of printed circuit board materials. By alloying the binder phase with Ru in combination with the use of fine grained Co-powder the properties have been improved.

Cemented carbide containing Ru as binder phase alone or in combination with the conventional Co and/or Ni is known in the art. For example, AT 268706 discloses a hard metal with Ru, Rh, Pd, Os, Ir, Pt and Re alone or in combination as binder phase. U.S. Pat. No. 4,574,011 discloses a hard metal composition for ornamental purposes with a binder phase of Co, Ni and Ru. GB 1309634 discloses a cutting tool with a Ru binder phase. GB 622041 discloses a hard metal composition a Co+Ru binder phase.

The routing of Printed Circuit Board materials requires a wide range of properties from the tool material in order for it to perform successfully. These include a hardness in excess of 2000 HV, a resistance to edge chipping that is best defined by a fracture toughness in excess of 8 MPam<sup>1/2</sup>, a resistance to chemical attack from the resins included in printed circuit boards and a sharp as possible a cutting edge. Some of these requirements conflict, for instance the high hardness tends to mean a reduced edge toughness. The new products for this application can, therefore, require a reduced WC grain size to produce a higher hardness with reduced toughness. However, if this is combined with an increase in cobalt content an increased toughness can be achieved for the same hardness. This also results in a sharper cutting edge, which is required.

The invention is primarily concerned with the addition of ruthenium to submicron grades of cemented carbide. The levels of addition vary between 5 and 35, preferably between 15 and 30, wt-% of the binder content with the best results obtained at about 25 wt-%. For best effects the cobalt used should be of the fine grain size cobalt powder having deagglomerated spherical grains of about 0.4  $\mu\text{m}$  average grain size and with a narrow grain size distribution. Preferably the cobalt powder is polyol cobalt. The cobalt contents to which this addition can be made should vary from 5–12%, preferably 5–8. The average WC grain size shall be <0.8  $\mu\text{m}$ , preferably <0.4  $\mu\text{m}$ . The cemented carbide of the invention is preferably a straight WC+Co grade but it may also contain <5 wt-% gammaphase.

In order to obtain the submicron WC grain size VC+Cr<sub>3</sub>C<sub>2</sub> is added. Because the Ru also acts as a mild grain growth inhibitor an addition of <0.9 wt % VC+Cr<sub>3</sub>C<sub>2</sub> is generally satisfactory. Particularly good results are obtained if the VC/Cr<sub>3</sub>C<sub>2</sub> ratio in wt % is 0.2–0.9, preferably 0.4–0.8, most preferably 0.6–0.7. Preferably sintering is performed using gas pressure sintering also referred to as sinter-HIP.

The invention also relates to the use of a cemented carbide with submicron WC grain size and with a binder phase containing 10–30 wt-% Ru as a tool for drilling/routing of printing circuit board materials.

The present invention further relates to a method of making a cemented carbide body comprising one or more hard constituents and a binder phase based on cobalt, nickel and/or iron by powder metallurgical methods milling pressing and sintering of powders forming hard constituents and binder phase whereby said binder phase contains 10–30 wt-% Ru. At least part of the binderphase powder consists of non agglomerated particles of spheroidal morphology of

## 2

about 0.4  $\mu\text{m}$  average grain size and with a narrow grain size distribution wherein at least 80% of the particles have sizes in the interval  $x \pm 0.2x$  provided that the interval of variation (that is  $0.4x$ ) is not smaller than 0.1  $\mu\text{m}$ .

The advantages offered by the ruthenium additions are as mentioned a further element of grain growth refinement, an increase in resistance to chemical attack and a strengthening of the binder phase without significantly affecting the edge toughness due to the increase in cobalt content used.

10

## EXAMPLE 1

Cemented carbide PCB-router according to the invention were made with the composition 1.9% Ru, 5.6% Cobalt the remainder, WC (0.2  $\mu\text{m}$  grain size), with about 0.7% (VC+Cr<sub>3</sub>C<sub>2</sub>) grain growth inhibitor. The material had a hardness of 2080 HV and a K1C of 8.75 MPam<sup>1/2</sup>.

For comparison the following PCB routers according to prior art were also made. One was 6% cobalt grade with 0.4  $\mu\text{m}$  WC with a hardness of 2000–2100 HV and one with the same hardness but with 5% cobalt and 0.5  $\mu\text{m}$  WC grain size.

The routers were ground to 2.4 mm dia and tested as follows:

Workmaterial: Copper clad 3 mm thick FR4 PCB, stacked three deep

Test 1: 30,000 RPM, 1.2 m/min feedrate, 150 m of cut

Test 2: 42,000 RPM, 2.2 m/min feedrate, 100 m of cut

In test 1 routers according to the invention reached 150 m of cut with 25% less average wear than the prior art routers which used 6% cobalt.

In test 2 routers according to the invention reached 100 meters of cut with acceptable levels of wear.

Routers according to prior art with 5% and 6% cobalt both fractured between 50 and 75 meters.

## EXAMPLE 2

2.4 mm dia routers according to the invention were made from cemented carbides with varying ruthenium contents as follows:

Composition 1: 1.0% Ru, 6.3% Co, 0.7 VC+Cr<sub>3</sub>C<sub>2</sub>, 0.2  $\mu\text{m}$  WC

Composition 2: 1.4% Ru, 6.0% Co, 0.7 VC+Cr<sub>3</sub>C<sub>2</sub>, 0.2  $\mu\text{m}$  WC

Composition 3: 1.9% Ru, 5.6% Co, 0.7 VC+Cr<sub>3</sub>C<sub>2</sub>, 0.2  $\mu\text{m}$  WC

The routers were tested as follows:

Workmaterial: Copper clad 3 mm thick FR4 PCB, stacked three deep

Conditions: 30,000 RPM, 1.2 m/min feed rate.

Machining until fracture.

Results:

1.0% Ru variant—205 m (Average of 4 cutters)

1.4% Ru variant—333 m (Average of 5 cutters)

1.9% Ru variant—366 m (Average of 7 cutters)

## EXAMPLE 3

Cemented carbide PCB microdrills according to the invention were made with the composition 2.2% Ru, 6.4% Co the remainder WC (0.4  $\mu\text{m}$  grain size), with about 0.8 % (VC+Cr<sub>3</sub>C<sub>2</sub>) grain growth inhibitor. The material had a hardness of 2001 HV and a K1C of 8% MPam<sup>1/2</sup>.

For comparison the following PCB microdrills according to prior art were made using 8% cobalt grade with 0.4  $\mu\text{m}$  WC with a hardness of 1900 HV.

**3**

The microdrills were tested and the wear measured. It was found that the prior art materials exhibited 10–15% less wear resistance and 10–15% less resistance to breakage during an increasing feed rate that started at 15  $\mu\text{m}/\text{rev}$  and increasing towards 70.

What is claimed is:

1. Cemented carbide comprising 5–12% Co binder phase, VC in an amount greater than zero,  $\text{Cr}_3\text{C}_2$  in an amount greater than zero, such that  $\text{VC}+\text{Cr}_3\text{C}_2$  is in an amount greater than zero and less than 0.9 wt. %, and remainder submicron WC wherein said binder phase further contains 10–30 wt-% Ru.

2. Cemented carbide according to claim 1, wherein the binder phase content is 5–8 wt-%.

**4**

3. Cemented carbide according to claim 1, wherein said binder phase further contains about 25 wt-% Ru.

4. A machining tool comprising cemented carbide with submicron WC grain size and with 5–12% Co binder phase containing 10–30 wt-% Ru, and VC in an amount greater than zero,  $\text{Cr}_3\text{C}_2$  in an amount greater than zero, such that  $\text{VC}+\text{Cr}_3\text{C}_2$  is in an amount greater than zero and less than 0.9 wt. %.

5. Cemented carbide according to claim 1, wherein the ratio of wt. % defined  $\text{VC}/\text{Cr}_3\text{C}_2$  is 0.2–0.9.

\* \* \* \* \*